

## UNITED STATES PATENT OFFICE

2,006,733

DENTAL INVESTMENT COMPOSITION AND  
PROCESS

Paul Francis Collins, Columbus, Ohio, assignor to  
The Columbus Dental Manufacturing Com-  
pany, Columbus, Ohio, a corporation

No Drawing. Application June 30, 1933, Serial  
No. 678,547

14 Claims. (Cl. 22—188)

The present invention relates to an investment composition for dental castings, and particularly for making dental castings in which a preshaped piece of precious metal or precious metal alloy is placed in an investment composition, and precious metal or precious metal alloy is cast upon the said inserted piece. The inserted piece may be a backing, a clasp, bridgework, dental plate, pin or the like. Hereinafter the term "precious metal" will be understood to include alloys containing one or more precious metals, with or without one or more non-noble metals.

In the process of casting, (which term is used in a broad sense to include also soldering together of a plurality of precious metal pieces, in making up artificial dentures and the like), it is customary to imbed a precious metal piece or a plurality of such metal pieces, in an investment composition, leaving preshaped spaces into which the precious metal is to be run, the investment composition being previously mixed up with water to form a mass of pasty consistency. The investment composition sets to a relatively hard mass, and subsequently is dried and heated, prior to the introduction of the new precious metal in a liquid state, to be cast onto the insets. It is customary to form the cavity into which the precious metal is to be poured, by attaching to the insets, wax which has the form desired in the cast metal. It is customary to heat up the mold thereby formed, sufficiently to thoroughly dry this out, and to melt out the wax, which wax may partly run out through a sprue hole provided, and/or some of the wax may be absorbed by the investment composition, after the latter has set, and during the heating operation. The heating of the mold may be carried to a rather high temperature, since by such procedure the mold is already hot before pouring in the molten precious metal, which latter is accordingly not chilled until it has completely filled the space previously occupied by the wax.

The investment composition usually employed contains a silicious base, for example finely ground quartz, sand and the like. The investment composition also contains a binder, usually plaster of Paris, or some other gypsum product, namely calcium sulphate, which of course becomes completely hydrated during the steps of mixing with water and air setting. Agents to retard or accelerate the setting or hardening, and/or to modify the plasticity of the wet mixture, may also be used, as is well known in the art.

The heating up of the molds may be performed in various ways, and it is not always convenient

for the dentist or the workers in the dental laboratory, to carefully control the temperature conditions in the molds, during the heating up and casting processes. The heating may be accomplished by placing the mold, after removal of the sprue pin or sprue pins, over a gas flame, or on a hot plate, or in an oven or in some other manner and usually it is a fact (although frequently not appreciated by the worker) that the atmosphere within the mold, and adjacent to the insets above referred to, may become reducing, when the material is subjected to a high temperature such as about 900° F. up to 1600° F., or higher, this reducing atmosphere being perhaps produced by the residues of the wax, or by the gas coming from the gas burner, when incompletely consumed, or from other causes. There is also liability of a more or less large portion of the calcium sulphate in the investment composition to be decomposed, in the presence of silica, liberating sulphur trioxide, which, in the reducing atmosphere sometimes forms free sulphur, or reduced sulphur compounds including calcium sulphide, hydrogen sulphide, carbon bisulphide, sulphur dioxide, and perhaps others, and this may cause deterioration of the piece or pieces of precious metal or precious metal alloy initially inserted into the investment composition, and against which it is desired to cast precious metal or precious metal alloy. It is also possible that sulphur compounds if present in the heating gas may produce or aid in producing the said deterioration.

The deterioration appears to be progressive, and appears to be much greater when temperatures higher than ordinary are employed, and when continued for a relatively long period. Ordinarily it has been practice in this type of casting, to use temperatures up to about 1500° F. continued for about an hour or more.

In accordance with the present invention, I may employ, as the basis of the investment composition, any of the usual investment compositions such as 18 to 50 parts of plaster of Paris or other calcium sulphate binder, and 50 to 82 parts of fine sand or other inert silicious material. With the said materials I employ a protective agent, as described below, for preventing deterioration of the precious metal and particularly for preventing deterioration of precious metal insets as described above.

The whole of the investment composition is preferably in a finely divided condition, so that 85% shall pass a number 200 sieve, 95% shall pass a number 100 sieve and 100% shall pass a

number 30 sieve. This screen analysis is generally accepted as standard, by the profession. Other materials such as asbestos fibers or other agent to impart strength, coloring matters as well known in the art, can be added if desired.

The protective agents which I have found to be most suitable are substances which are capable of readily combining with sulphur, to produce sulphides.

- 10 I have found that by the addition, as protective agents, of the metals copper, nickel, cobalt, iron, molybdenum or silver, (as free metals, i. e. in the pure metallic state) or alloys of these metals among themselves, or with zinc or alloys of one 15 or more of these metals with other metals, or the oxides of copper, nickel, cobalt, or silver, in the amount of about 7 to 15% of the total investment composition, it is entirely possible to protect metal insets from deterioration, even 20 when heated in the mold for a long period such as 6 to 8 hours. These substances are the most effective, for producing the said effect, of all the many substances with which I have experimented. Smaller amounts of the above 25 mentioned materials can be added, if the heating is to be continued for not more than about one and a half to two hours, as well as 7 to 15% of an oxide of manganese, such as manganese dioxide, chromium oxide, molybdenum trioxide, 30 molybdenum sesquioxide, molybdenum dioxide, cuprous oxide, or zinc oxide. If it is necessary to afford protection to the precious metal insets for only a much shorter period, such as 30 minutes to one hour at high temperature, metals such as chromium or manganese, can be employed, also more than 7% of ferric oxide or ferroferric oxide. These materials can be used in the amount of 7 to 15% or more, or in place 35 of these materials, smaller quantities of the 40 materials of the first and second groups above mentioned can be employed. About 3 to 5% of powdered chromium oxide is also to some extent useful in preventing or retarding injury to the metal insets.
- 45 In place of the metals or oxides, I may employ certain other materials, for example carbonates, oxalates or other organic acid salts of the metals, which upon heating to the temperatures above stated will decompose to leave oxide 50 or metal. I find also that chlorides and other haloid acid salts of the above metals can be used in place of the metals or oxides. However the use of the haloid salts does not appear to be of any particular advantage over the use 55 of the metals or oxides, and in certain cases they are not as satisfactory. I find also that certain alkaline earth metal halides (e. g. example strontium chloride) give fairly good results. The metal tungsten or its oxide or nitrate or 60 chloride also can be used. Nitrates of all of the metals referred to above can be suitably employed, these of course giving oxides during the heating operation. I have found also that difficultly reducible salts of the acids which contain amphoteric metals in the acid radical can 65 suitably be employed, for example sodium molybdate, sodium tungstate, both of which were found to give fairly good results. The above mentioned salts, as will be noted, do not contain sulphur. I believe that sulphur-containing salts would not be useful for the purposes indicated. Insoluble salts (e. g. carbonates) are usually preferable to soluble salts.
- 70 Of the first class of substances above referred 75 to, I preferably employ at least 7%, and up to

15% or more of the protective substance, if it is desired to prevent deterioration during the heating period at high temperature for 6 hours. If the heating is to be continued for only about 2 hours or less, about 2 to 7% of the first class 5 of materials can be found sufficient in most cases.

The amount of the protective material to be added can vary between rather wide limits, depending upon the composition of the embedded 10 metal to be protected, the temperatures which are to be employed in heating up and casting, and the length of time taken to complete the operation. Quantities from 0.5% up to 40% of the entire investment composition can be employed. With most of the cases I would recommend the use of over 5% and not substantially over 25% of the protective agent, for giving most satisfactory results. With iron oxide I would preferably employ from 10 or 12% up to 20 25 or 25%.

The protective agent may be used in the investment composition as an aggregate, as a granular material or preferably as a pulverized material. The pulverized material is preferably 25 graded from 100 to 400 mesh. It is best thoroughly mixed with the investment composition, for example by grinding or mixing the entire mass together or by grinding or mixing some of the investment material (e. g. a small portion of 30 the sand or quartz) with the protective agent, then adding this to the remainder of the investment composition and grinding or mixing the final batch. It is usually advisable to use the protective agent in a very fine powder and to 35 very thoroughly and uniformly mix this with the remaining constituents of the investment composition. When employing metals in the elementary form, or alloys of metals the protective 40 agent will function satisfactorily if used in the form of small strips or pieces of foil placed around and in proximity to the metal insets, but such is not the preferred form.

In making up the composition, it will be understood that a small amount of a highly active 45 protective agent produces a result equivalent to a larger amount of a less active agent.

As an alternative mode of procedure, the operator could dissolve the protective agent in the water, or mix the protective agent with the water, 50 if not soluble therein, and use this water for mixing with the investment composition proper, in such proportions as indicated above. I consider the use of the protective agent in very finely divided condition, thoroughly mixed with 55 the remainder of the investment composition to be the most practical method of applying the invention.

I give the following examples, purely by way of illustration and without in any sense restrict- 60 ing the invention thereto.

#### Example 1

65% of fine sand, mixed with 22% of calcined gypsum as a binder, and 13% of a mixture of 65 equal parts of finely powdered metallic nickel and finely powdered metallic copper. This particular composition has been found to afford adequate protection to precious metal tooth backings composed of an alloy of gold, platinum, 70 palladium and silver, for a period of 8 hours, at a temperature much above the melting point of tin. Alloys containing at least two of the above named metals together with common base metals such as copper, nickel, etc., in the form 75

of insets as above described, are completely protected over all practical ranges of heat treatment commonly used in making dental investments.

5 *Example 2*

63 parts of silica, 20 parts of plaster of Paris (or other calcium sulphate binder) and 17 parts of a mixture of equal quantities of zinc oxide and cuprous oxide. This composition has been found to prevent deterioration of the metal backings noted above, for periods up to 2 hours.

10 *Example 3*

15 66 parts of silica, 22 parts of plaster of Paris (or other calcium sulphate binder) and 12 parts of manganese dioxide. This composition has been found to be an effective protective agent, under conditions specified above, for periods up to 20 20 45 minutes or so.

25 The terms "silica" and "siliceous base" are used herein to include sand, flint, quartz, cristobalite, and equivalent materials, reduced to the desired degree of fineness suitable for investment composition.

30 The above mentioned forms of silica are dense, compact or substantially non-porous, as compared with diatomaceous earth or kieselguhr, which latter material has been proposed in certain prior art in foundry molding, of copper and analogous metals, to impart a high degree of porosity to the mold. I do not use kieselguhr, but preferably use quartz, sand or similar materials as the siliceous filler. The dense silica 35 has been exclusively used in the actual practice heretofore, as the refractory oxide component of dental investment compositions.

40 As stated in the parent application, 642,317 (now Patent 1,953,075) the investment composition should have such thermal expansion properties as to counteract for shrinkage of gold on cooling the casting to room temperature.

45 As was originally stated in said parent case, "While the general proportions of the ingredients mainly used have been stated, manufacturers in the past have employed the main materials in varying proportions in attempts to meet the varying expressed requirements of the dental profession, such as the time required for the plastic 50 mass to air set, the expansion produced while air setting, the thermal expansion produced during heat treatment, the compressive strength at service temperature, and the degree of coarseness or fineness of the materials."

55 With diatomaceous earth or kieselguhr used as the principal siliceous content of the investment composition, the desired thermal expansion properties would be lost, due to the porous character of the said diatomaceous earth. Quartz and silica sand are well known to be crystalline forms of silica, whereas kieselguhr is a non-crystalline product of life processes. In certain of the appended claims I use the terms "dense" or "substantially non-porous" to cover specifically such siliceous materials as are used herein.

60 I have referred above to injury to metal insets caused, I believe, by the action of sulphur or reduced sulphur compounds derived from the decomposition of the calcium sulphate binder in the presence of silica in the investment composition. In some cases sulphur derived from the gas used in the gas burner may also cause injury to the metal insets, as also sulphur or perhaps other deleterious substances produced from substances 65 added as a retarder or accelerator for the calcium

sulphate binders, or added to regulate the set of the composition as a whole.

70 The preferred metals, to be used, in the form of metals or oxides or easily reducible sulphur-free salts, as protective agents are the following (with atomic weights given approximately) V=51, Cr=52, Mn=55, Fe=56, Co=59, Ni=59, Cu=63, Zn=65.4, Mo=96, Ag=108, W=184.

75 It will be understood that there are many other metals or elements which are capable of combining at some temperatures, with sulphur in a reduced condition, but many of these would be impractical for one reason or another. As examples, the following may be mentioned:

80 Such metals as lead, tin, cadmium, antimony, bismuth, caesium, gallium, indium and perhaps others, melt at temperatures commonly used in heating the investment and might injure the precious metals used in the process. Arsenic and osmium, when heated, may evolve offensive or 85 poisonous vapors or fumes. Uranium, thorium, radium and some others are radio-active. Thallium is poisonous. Mercury is poisonous and is a liquid which would be extremely harmful to precious metals. Magnesium and certain other 90 metals would react with water to be used with the investment composition, and would oxidize objectionably even before adding the water. Aluminum, gold, platinum, boron, osmium and titanium do not readily combine with free sulphur to form stable sulphides. No claim is made herein to the addition of the metals mentioned in this paragraph or the simple salts or oxides thereof, to investment compositions of the type 95 set forth, as the protective reagent.

100 The metals which I use herein are all metals which form stable sulphides. The sulphides of most of these metals are in fact so stable that they occur in nature as minerals. The metals, in the metallic condition mostly melt at temperatures above the highest temperatures commonly used in the investment process (up to about 1500-1600° F).

105 The metals whose atomic weights are listed above, furthermore, are all classified as "heavy" metals" (i. e. they have a specific gravity above 5) and thereby they are distinguished from "light metals" such as alkali metals, alkaline earth metals, aluminum, magnesium, etc. "Heavy metal" as used herein (as in accepted books on 110 chemistry) is to be understood as meaning a specific gravity above 5.

115 The present application is in part a continuation of my copending application Ser. No. 642,317, filed November 11, 1932, (now Patent 1,953,075). In said copending patent, I have claimed the application to investment compositions of the present type, of oxides of the alkaline earth metals (Ca, Ba and Sr) and of aluminum. No claim is made herein, to such subject matter, 120 nor the application of metallic aluminum.

125 My researches indicate that all of the metals chromium, copper, manganese, iron, cobalt, nickel, molybdenum, silver and tungsten, and the oxides of all of these metals, have a substantial 130 protective effect, but that some of these are far more effective than others. Metallic zinc as such is fairly effective, zinc alloys and easily reducible sulphur-free zinc salts also can be used. Zinc oxide is quite satisfactory. Vanadium in 135 the metallic form is quite satisfactory but is highly expensive. Vanadium oxide is less satisfactory than the metal. Mixtures of two or several of these can also be used, as well as alloys of the above metals with each other or with other 140

(apparently inert) metals, so far as these other metals are not injurious.

I have herein above described the use of metals of the group which have atomic weights (in round numbers) between 52 and 63, (or stated proportions of these metals) as protective agents in the investment composition. These metals can be used in the conditions above described, i. e. (a) in the metallic condition, (b) as oxides, 10 (c) in the form of alloys, (d) in the form of those sulphur-free salts (e. g. nitrates, carbonates, oxalates or other organic acid salts which upon heating to temperatures not higher than are commonly used in the investment process, are 15 decomposed to form free metals or oxides) and (e) halides (e. g. chlorides) which are not objectionably volatilized at temperatures commonly used in the investment process.

I claim:—

20 1. A dental molding composition comprising a siliceous filler, calcium sulphate and a heavy metal substance, said substance being selected from the group of metalliferous materials consisting of sulphur-binding metals either in a metallic form or in the form of an easily reducible sulphur-free compound, said heavy metal substance being capable of combining with sulphur at between 600° F. and 1800° F., to form a stable sulphide, said heavy metal substance being substantially harmless to precious metal dental alloys at said temperature, and substantially non-volatile at said 25 temperature.

30 2. A dental investment composition composed largely of compact refractory oxide filler, and a calcium sulphate binder, which investment composition contains a protective reagent which is a heavy-metal-containing metalliferous material capable of readily combining with sulphur in a reduced condition, at the temperatures normally 35 used in making dental products by the investment process, said metalliferous material containing a metal selected from the group consisting of chromium, manganese, iron, cobalt, nickel, copper, molybdenum, silver and tungsten, in a metallic 40 condition or in the form of an easily reducible sulphur-free compound.

45 3. An investment composition, of the calcium-sulphate-containing type which contains non-porous silica as a large constituent, containing, as a protective reagent, an easily reducible oxide of a metal selected from the group consisting of chromium, manganese, iron, cobalt, nickel, copper, molybdenum, silver and tungsten, in an amount capable of reacting with reduced sulphur compounds produced from said calcium sulphate during the use of said investment composition.

50 4. An investment composition as in claim 1, in which the amount of said reagent is between about 2% and 25%, based upon the weight of the entire investment composition, but the amount being insufficient to destroy the strength and thermal expansion properties of the casting investment.

55 5. A dental investment composition consisting principally of a substantially non-porous refractory siliceous filler and a calcium sulphate binder and containing a reagent which is capable of reacting with sulphur liberated from the calcium sulphate binder, said reagent being an easily reducible sulphur-free salt of a sulphur-binding metal, as described.

60 6. A dental investment composition of the type composed mostly of a calcium sulphate binder and a refractory oxide, which contains as a protective reagent, about 2 to 15% of copper as an easily 65

reducible compound or as free metal, which protective reagent is in the form of a fine powder.

7. A dental investment composition of the type composed mostly of a calcium sulphate binder and a refractory oxide, which contains as a protective reagent, about 2 to 15% of nickel as an easily reducible compound or as free metal, which protective reagent is in the form of a fine powder.

8. A dental investment composition of the type composed mostly of a calcium sulphate binder and a refractory oxide, which contains as a protective reagent, about 2 to 15% of cobalt as an easily reducible compound or as free metal, which protective reagent is in the form of a fine powder.

9. A dental molding composition comprising a siliceous filler, calcium sulphate and a metalliferous material which is a heavy-metal-stable-sulphide-forming substance, either in the metallic condition or in the form of an easily reducible sulphur-free compound, said substance being capable of combining with reduced sulphur produced under reducing conditions from the calcium sulphate at a temperature between 600° F. and 1800° F., which substance is non-volatile at said temperature, and which substance is harmless to precious metal dental alloys, at said temperatures, the said combining reaction rendering the sulphur non-injurious with respect to precious metal alloys used in making dental castings, the amount of said substance being enough to prevent harmful absorption of sulphur by said precious metal.

10. A method of casting precious metal upon a preshaped precious metal alloy inset, which comprises embedding such preshaped inset in a moistened investment as set forth in claim 9, allowing said moistened investment to set and harden, thereafter heating said investment to about 600° to 1800° F., until sufficiently dehydrated, and casting free precious metal in contact with said inset.

11. An investment composition which comprises a mixture of about 50 to 82 parts of a dense siliceous filler and about 18 to 50 parts of a calcium sulphate binder; in which is incorporated a protective reagent in the form of a 100 to 440 mesh powder in the amount of 2 to 25% of the entire investment composition, the amount of said reagent being enough to prevent harmful absorption of sulphur by the precious metal, said reagent being capable of combining with reduced sulphur derived from the calcium sulphate binder, at temperatures between 600° F. and 1800° F. to form a stable sulphide, and being selected from the herein described group of sulphur-binding metals consisting of chromium, manganese, iron, cobalt, nickel, copper, molybdenum, silver and tungsten, either in a metallic form, or in the form of an easily reducible sulphur-free compound.

12. An investment composition which comprises a mixture of about 50 to 82 parts of a dense siliceous filler and about 18 to 50 parts of a calcium sulphate binder, in which is incorporated a protective reagent in the amount of 2% to 25% of the entire investment composition, the amount of said reagent being enough to prevent harmful absorption of sulphur by the precious metal, said reagent being capable of combining with reduced sulphur derived from the calcium sulphate binder, at temperatures between 600° F. and 1800° F., to form a stable sulphide, and being selected from the herein described group of sulphur-free metalliferous substances consisting of sulphur-binding metals selected from the group

consisting of chromium, manganese, iron, cobalt, nickel, copper, molybdenum, silver and tungsten, either in a metallic condition or as an easily reducible sulphur-free compound.

5 13. A method of protecting preshaped pieces of precious metals or alloys thereof when being heated for a protracted period in an investment composed of a composition including calcium sulphate which comprises the step of incorporating with the investment composition a protective reagent as defined in claim 11.

10 14. That step in the casting of metals which comprises forcing said metal in a molten state into a preshaped cavity in a hardened invest-

ment composition while said hardened investment composition is at between 600° and 1800° F., said investment composition being composed of a refractory oxide and calcium sulphate, and a metalliferous substance containing a heavy metal selected from the group consisting of sulphur-binding metals either in a metallic form or in the form of an easily reducible sulphur-free compound, said group of metals being capable of combining with reduced sulphur as liberated 10 from the calcium sulphate between the aforesaid temperatures.

PAUL FRANCIS COLLINS.